

## UNITED STATES PATENT OFFICE

2,589,607

## MATCH STRIKING COMPOUNDS

Herbert Ellern, Ferguson, Mo., assignor to Universal Match Corporation, St. Louis, Mo., a corporation of Delaware

No Drawing. Application March 9, 1946,  
Serial No. 653,445

3 Claims. (Cl. 52--28)

1

This invention relates in general to certain new and useful improvements in match striking compounds and the methods of manufacturing and applying the same.

In the manufacture of so-called safety matches, commonly referred to in the match industry as strike-on-box matches, it has been accepted practice to prepare a striking compound containing as active chemical ingredients red phosphorus and finely powdered glass in a relatively thin non-viscous aqueous suspension and apply such compound in a thin film layer upon one of more of the external surfaces of the box or package in which the matches are contained. The user, upon removing a match, may draw the match-head sharply across the striking surface to produce chemical interaction between the phosphorus in the striking compound and the chlorate in the match-head. Existing striking compounds contain such a large percentage of water that the drying time thereof is extremely long and the production of match packages seriously attenuated. Efforts to speed up drying by increasing the temperature of the drying tunnels or by increasing the flow of air which is circulated therethrough cause the striking compound to dry with a hard, smooth, and relatively friction-free surface which is practically useless for match-striking purposes.

It is, therefore, an object of the present invention to provide a new and improved striking compound which is simple and economical to prepare and compound, which has relatively low viscosity at a very low solvent content, and which possesses remarkably accelerated drying properties.

It is a further object of the present invention to provide a striking compound which may be speedily applied and will dry rapidly in the formation of a flat, non-glazed, and highly sensitive striking surface.

It is an additional object of the present invention to provide a striking compound of the type stated which will dry rapidly and may be safely subjected to increased drying temperatures without the production of a glazed surface and without blistering or cracking.

And with the above and other objects in view, my invention resides in the novel processes and compositions of matter presently described and pointed out in the claims.

Broadly speaking, my invention comprises the formation of a striking compound by the intermixture of red phosphorus, finely powdered glass, and other similar inert ingredients and modified casein, that is to say, casein which has been solubilized in the presence of limited amounts of water and caustic soda with the further optional addition of water compatible organic agents capable of lowering the viscosity of the casein solution. The modified casein solution is first made up and allowed to stand for a relatively

2

short time until it has reached complete uniformity, smooth consistency, and satisfactory viscosity. Thereupon, the phosphorus and inert ingredients are added to the casein solution and the batch is thoroughly agitated until uniformly mixed. The resulting striking compound has the consistency of a free-flowing slurry and may be applied at a temperature of approximately 130° F. to the surface of match boxes or to sheets of cardboard stock used in the manufacture of match boxes in the usual manner.

After application, the coated paper stock or match boxes, as the case may be, is immediately passed beneath elongated radiant heating elements adapted to focus sharply upon the coated strip or area and produce a very rapid elevation of temperature directly within the coating itself, with the result that the coating is dried in five to thirty seconds. In actual practice, the coated web of paper stock or other coated material is moved at a relatively rapid rate of lineal travel beneath a series of radiant heat elements extending over a substantial lineal distance in order to maintain adequate production capacity in the machinery, although it should be understood that, for specific applications, it is possible to move the web at a comparatively slower speed over relatively shorter distances.

By way of illustration and not by way of limitation, it has been found that the following specific formulae will produce excellent results:

*Example I*

|                   | Parts by Weight |
|-------------------|-----------------|
| Casein            | 12              |
| Caustic soda      | 1               |
| Red phosphorus    | 50              |
| Whiting           | 5               |
| Zinc oxide        | 5               |
| Powdered charcoal | 3½              |
| Powdered glass    | 23½             |
| Water             | 45              |
| Ethylalcohol      | 15              |

*Example II*

|                | Parts by Weight |
|----------------|-----------------|
| Casein         | 12              |
| Caustic soda   | 1½              |
| Red phosphorus | 45              |
| Zinc oxide     | 5               |
| Powdered glass | 36½             |
| Water          | 60              |

*Example III*

|                         | Parts by Weight |
|-------------------------|-----------------|
| Casein                  | 11              |
| Caustic soda            | 2               |
| Red phosphorus          | 45              |
| Zinc oxide              | 8               |
| Carbon black            | 2               |
| Black antimony sulphide | 32              |
| Water                   | 30              |
| Ethylalcohol            | 15              |

Generally speaking, I have found that striking compounds made in accordance with the present invention can be formulated with a water content ranging from 20% to 40% by weight and, even in such dilutions as 20% by weight of water, at which dilution the compound has a consistency of a heavy paste, the results upon drying are completely satisfactory and uniform. The ability to compound the solution in such heavy paste form makes it possible to apply such striking compound by methods of intaglio printing. Furthermore, it should also be pointed out that the alcohol, which is additionally employed as has been mentioned above in some of the specific examples set forth, is not present in sufficient quantity to act as a vehicle or diluent in and of itself, but is actually a viscosity reducing agent producing marked lowering of viscosity. If desired, other aliphatic alcohols or acetone may be substituted for ethylalcohol for this purpose. In addition, it may be stated that a small quantity of furfural or furfuryl alcohol may be added to the modified casein solution during its preparation to counteract the tendency of the casein solution to gel upon standing. The addition of these latter ingredients is not necessary unless manufacturing conditions require that the casein solution be allowed to stand over protracted periods of time.

In preparing the modified casein solution, I have also found that it is possible to substitute potassium hydroxide, lithium hydroxide, and aliphatic amines, such as ethylene diamine, for example, or combinations of these ingredients.

It should be understood that changes in the methods, compositions, percentages, and combinations above set forth may be made without departing from the nature and principle of my invention.

Having thus described my invention, what I claim and desire to secure by Letters Patent is:

1. A striking compound having the following constituency:

| Parts by Weight   |     |  |
|-------------------|-----|--|
| Casein            | 12  |  |
| Caustic soda      | 1   |  |
| Red phosphorus    | 50  |  |
| Whiting           | 5   |  |
| Zinc oxide        | 5   |  |
| Powdered charcoal | 3½  |  |
| Powdered glass    | 23½ |  |
| Water             | 45  |  |
| Ethylalcohol      | 15  |  |

2. A striking compound having approximately the following constituency:

| Parts by Weight   |     |  |
|-------------------|-----|--|
| Casein            | 12  |  |
| Caustic soda      | 1   |  |
| Red phosphorus    | 50  |  |
| Whiting           | 5   |  |
| Zinc oxide        | 5   |  |
| Powdered charcoal | 3½  |  |
| Powdered glass    | 23½ |  |
| Water             | 45  |  |
| Ethylalcohol      | 15  |  |

3. A striking compound consisting essentially of an alkaline caseinate, red phosphorus, zinc oxide, powdered glass and water and in which compound the water constitutes from 20% to 40% of the total mixture.

HERBERT ELLERN.

#### REFERENCES CITED

The following references are of record in the file of this patent:

#### UNITED STATES PATENTS

| Number    | Name     | Date          |
|-----------|----------|---------------|
| 83,633    | Austin   | Nov. 3, 1868  |
| 579,913   | Allday   | Mar. 30, 1897 |
| 949,920   | Swoboda  | Feb. 22, 1910 |
| 1,206,827 | Fairburn | Dec. 5, 1916  |
| 1,341,012 | Dixon    | May 25, 1920  |
| 1,718,358 | Jordan   | June 25, 1929 |
| 1,773,400 | Light    | Aug. 19, 1930 |

#### FOREIGN PATENTS

| Number  | Country       | Date          |
|---------|---------------|---------------|
| 420,653 | France        | Nov. 29, 1910 |
| 248,115 | Germany       | June 11, 1912 |
| 191,906 | Great Britain | Jan. 25, 1923 |
| 314,852 | Great Britain | Nov. 28, 1929 |
| 458,515 | Great Britain | Dec. 22, 1936 |
| 2,273   | Australia     | June 21, 1927 |

#### OTHER REFERENCES

Sutermeister, "Casein," 1939, Pages 241-243, 285 and 286.  
 Sutermeister et al.: "Casein and Its Industrial Applications," pages 244, 355, 356, 392, 393, second edition, Reinhold Publishing Co. (1939).